

2,868,730

## INSULATING OILS

James Campbell Wood-Mallock, Macclesfield, and Fred Hughes, Stretford, England, assignors to Manchester Oil Refinery (Holdings) Limited, Manchester, England

No Drawing. Application March 28, 1955  
Serial No. 497,391

Claims priority, application Great Britain  
March 30, 1954

2 Claims. (Cl. 252—63.7)

The present invention concerns improvements in insulating oils such as, for example, transformer oils, which are mineral oils used in transformers for cooling purposes, usually possessing a flash point over 160° C., having little or no volatility at 100° C. and free from moisture.

Transformer oil functions as a fluid di-electric medium and as a heat transfer fluid and in general any deterioration in the oil occurs slowly and progressively over a large number of years. Deterioration occurs as a result of access of oxygen to the system and contact of the oil insulant with the constructional materials of the transformer at the relatively high service temperature. Access of oxygen can be limited to some extent by the provision of conservators and the life of the oil insulant in such instances is usually long but in a number of cases and particularly with ventilated transformers severe failure occurs within a relatively short time.

It is known that of the materials normally used in the construction of a transformer the one which accelerates deterioration by oxidation to the greatest extent is copper. It has been shown that under certain conditions copper induces acidity development in the oil almost immediately so that the neutralisation number rises by 0.04 mg. KOH/g. in the first ten days. Thus the conditions for solubilising copper in the insulating oil, namely, acidity and contact with the metal, do exist and although the rate of solution is extremely slow it is known that at low concentrations of a fraction of a part per million copper is extremely active and can catalyse oxidation. We have determined the copper content of a number of used transformer oil samples by the ion exchange technique described by H. Buchwald and L. G. Wood (Anal. Chem. 1953, 25, 664). It was found that copper was present to the extent of between 0.16 and 4 parts per million.

The use of anti-oxidants and metal de-activators in motor spirit has previously been proposed, but it has been found that no substantial benefits are obtained when the commercially available copper de-activators such as the tertiary organic amines Tenamene "60" (di-salicyl propylene diamine in toluene) and Nonoxol "CD" (di-salicyl ethylene diamine), and many other proposed de-activators are added to transformer oil. Such additions cause an appreciable increase in the rate and amount of copper solubilised in most cases and do not result in any large reduction in sludge formation or acid development when the oil is subjected to the British Standard Specification 148—1951 accelerated oxidation test, described in "Insulating Oil for Transformers and Switch-gear," published by British Standards Institution, 24-28 Victoria Street, London, S. W. 1, England, even when anti-oxidants are also present.

In contrast therewith, it has now been found that substantial benefits are obtained by the addition to transformer and other insulating oils of certain aromatic primary amines in combination with an anti-oxidant selected from the group consisting of phenyl-alpha-naphthylamine and phenyl-beta-naphthylamine.

2  
The aromatic primary amines are those of the general formula



5  
10 wherein R<sup>1</sup>, R<sup>2</sup>, R<sup>3</sup> and R<sup>4</sup> are similar or dissimilar, are selected from H and alkyl radicals containing up to 12 carbon atoms, and together do not contain more than 24 carbon atoms, and X is NH<sub>2</sub> or COOH.

15 Examples of these aromatic amines are o-phenylene diamine, anthranilic acid and their nuclear substituted alkyl derivatives. The anti-oxidant may be either phenyl- $\alpha$ -naphthylamine or phenyl- $\beta$ -naphthylamine.

The preferred amount of metal deactivator present in the insulating oils of the invention is from 0.001 to 0.1% by weight. The preferred content of anti-oxidant is from 0.01 to 0.25% by weight.

20  
25 Particularly valuable insulating oils in accordance with the invention are transformer oils containing at least 0.03% of phenyl- $\beta$ -naphthylamine and at least 0.02% of anthranilic acid.

30 The presence of the aromatic primary amine with the anti-oxidant in the insulating oils of the invention not only reduces the harmful effect of copper but also of other metals, e. g. iron, with which the oil may come into contact during use.

35 The solubilising effect on copper of insulating oils treated according to the present invention and their stability towards deterioration by oxidation have been assessed by tests simulating service conditions and by the B. S. 148—1951 accelerated oxidation test which requires the use of a clean pure hydrocarbon (mineral) oil. The results are set out below together with comparative results for the commercially available metal deactivators Tenamene "60," Nonoxol "CD" and Accolube "76."

40  
45 The test simulating service conditions in a ventilated transformer consisted in subjecting 200 square centimetres of a copper surface, cleaned according to B. S. 148—1951, to the action of 200 millilitres of oil which is stirred at 70° C. for three days in a thermostatically controlled bath and the amount of copper which dissolved in the insulating oil was determined by the method of Buchwald and Wood referred to above.

50  
55 In the tests the insulating oils used were transformer oil as currently marketed (B. S. 148—1951), similar oil after being subjected to further treatments known in this art and transformer oil B. S. 148—1951 treated according to the present invention. The additive "P. B. N." referred to in the tables below is the anti-oxidant phenyl- $\beta$ -naphthylamine. All percentages quoted are percentages by weight.

|       | Insulating Oil                                                                                               | Copper, p.p.m., after 3 days at 70° C. |
|-------|--------------------------------------------------------------------------------------------------------------|----------------------------------------|
| 60    |                                                                                                              |                                        |
| a.    | B. S. 148—1951 Transformer Oil Batch Type A                                                                  | 1.20                                   |
| b.    | B. S. 148—1951 Transformer Oil treated conventionally:<br>Type A after 3 x N NaOH washes +3% activated earth | 0.25                                   |
|       | Type A after 3 x N NaOH washes, dehydrated                                                                   | 0.80                                   |
|       | Type A distilled from solid NaOH                                                                             | 0.75                                   |
| 65 c. | B. S. 148—1951 Transformer Oil with Additives:<br>Type A +0.1% P. B. N.                                      | 0.30                                   |
|       | Type A +0.1% P. B. N. +0.02% Tenamene "60"                                                                   | 3.95                                   |
|       | Type A +0.1% P. B. N. +0.02% Nonoxol "CD"                                                                    | 1.10                                   |
|       | Type A +0.1% P. B. N. +0.02% ethylene diamine                                                                | 1.20                                   |
|       | Type A +0.1% P. B. N. +0.02% anthranilic acid                                                                | 0                                      |
| 70    | Type A +0.1% P. B. N. +0.02% o-phenylene diamine                                                             | 0                                      |
|       | Type A +0.1% P. B. N. +0.0024% Accolube "76"                                                                 | 3.00                                   |

(Accolube "76" is a known deactivator consisting of zinc hexyl dithio-phosphate.)

It will be seen that under these test conditions transformer oil B. S. 148-1951 will dissolve 1.2 parts per million of copper and that the conventional treating methods may reduce this to 0.25 part per million, whereas the addition of phenyl-beta-naphthylamine as an anti-oxidant and either anthranilic acid or o-phenylene diamine according to the invention prevents the solution of copper. The amount of copper dissolved when phenyl-beta-naphthylamine and ethylene diamine are used according to the invention is identical with the amount dissolved in untreated oil. It has to be pointed out, however, that the method of analysis of Buchwald and Wood determines the total soluble copper whether present as a complex with a deactivator or as a copper soap of the acids developed when copper is contacted with insulating oil at elevated temperatures.

The results obtained on carrying out the accelerated oxidation tests according to the method of B. S. 148-1951 are given below:

| Insulating Oils                                          | Sludge, Percent | Acid Development, mg. KOH/g. |
|----------------------------------------------------------|-----------------|------------------------------|
| <i>a. Base Oils:</i>                                     |                 |                              |
| B. S. 148-1951 Transformer Oil Batch, Type B             | 0.92            | 1.15                         |
|                                                          | 0.89            | 1.15                         |
| B. S. 148-1951 Transformer Oil Batch, Type A             | 0.81            | 1.26                         |
|                                                          | 0.86            | 1.28                         |
| <i>b. B. S. 148-1951 Transformer Oil with Additives:</i> |                 |                              |
| Type B+0.1% P. B. N.                                     | 1.38            | 1.43                         |
|                                                          | 1.50            | 1.50                         |
|                                                          | 0.37            | 0.65                         |
|                                                          | 0.35            | 0.63                         |
|                                                          | 0.60            | 0.88                         |
| Type B+0.02% ethylene diamine                            | 0.70            | 0.86                         |
| Type B+0.02% anthranilic acid                            | 0.14            | 0.24                         |
| Type B+0.1% P. B. N.+0.02% ethylene diamine              | 0.10            | 0.21                         |
| Type B+0.1% P. B. N.+0.02% anthranilic acid              | 0.09            | 0.19                         |
|                                                          | 0.07            | 0.22                         |
| Type A+0.1% P. B. N.                                     | 0.59            | 1.18                         |
| Type A+0.1% P. B. N.+0.02% Tenamene "60"                 | 0.96            | 1.16                         |
| Type A+0.1% P. B. N.+0.01% ethylene diamine              | 0.99            | 1.18                         |
| Type A+0.1% P. B. N.+0.01% Nonoxol "CD"                  | 0.27            | 0.53                         |
|                                                          | 0.34            | 0.54                         |
| Type A+0.1% P. B. N.+0.02% anthranilic acid              | 0.14            | 0.25                         |
| Type A+0.1% P. B. N.+0.01% Nonoxol "CD"                  | 0.15            | 0.30                         |
|                                                          | 0.57            | 0.94                         |
| Type A+0.1% P. B. N.+0.02% o-phenylene diamine           | 0.72            | 1.26                         |
|                                                          | 1.16            | 2.72                         |
|                                                          | 1.06            | 2.80                         |
|                                                          | 0.15            | 0.38                         |
|                                                          |                 | 45                           |

It will be seen that the combination of phenyl-beta-naphthylamine and the copper deactivators, anthranilic acid and o-phenylene diamine gave the best results in reducing sludge and acid development.

5 We claim:

1. A new insulating transformer oil composition consisting essentially of a mineral transformer oil and: (a) from about 0.001 to about 0.1% by weight of a compound selected from the group consisting of anthranilic acid and o-phenylene diamine, (b) from about 0.01% to 10 about 0.25% by weight of a compound selected from the group consisting of phenyl-alpha-naphthylamine and phenyl-beta-naphthylamine.

15 2. A new insulating transformer oil composition consisting essentially of a mineral transformer oil, and: (a) a compound selected from the group consisting of anthranilic acid and o-phenylene diamine in an amount effective to function as a metal deactivator in the transformer oil, and (b) a compound selected from the group 20 consisting of phenyl-alpha-naphthylamine and phenyl-beta-naphthylamine in an amount effective to function as an anti-oxidant in the transformer oil.

#### References Cited in the file of this patent

#### UNITED STATES PATENTS

|    |           |          |                |
|----|-----------|----------|----------------|
| 25 | 1,973,676 | Voorhees | Sept. 11, 1934 |
|    | 1,988,299 | Clark    | Jan. 15, 1935  |
|    | 2,354,252 | Fraser   | July 25, 1944  |
|    | 2,369,090 | Trautman | Feb. 6, 1945   |
|    | 2,530,650 | Chenicek | Nov. 21, 1950  |
|    | 2,573,779 | Walters  | Nov. 6, 1951   |